

March 31, 1925.

1,531,858

J. W. GALVIN

METHOD OF AND APPARATUS FOR MAKING ELECTRIC STEEL

Filed April 28, 1920

2 Sheets-Sheet 1

*Fig. 1.*



*Fig. 2.*



WITNESS.

*Gustav Jenzinger.*

INVENTOR.  
James W. Galvin  
BY  
*Symonoff & Lechner*  
ATTORNEYS.

March 31, 1925.

1,531,858

J. W. GALVIN

METHOD OF AND APPARATUS FOR MAKING ELECTRIC STEEL

Filed April 28, 1920

2 Sheets-Sheet 2

Fig. 3.



Fig. 4.



WITNESS.

Gustav Genzlinger.

INVENTOR.  
BY James W. Galvin  
Spencer & Dechner  
ATTORNEYS.

Patented Mar. 31, 1925.

1,531,858

# UNITED STATES PATENT OFFICE.

JAMES W. GALVIN, OF SPRINGFIELD, OHIO, ASSIGNOR OF ONE-HALF TO JOHN GALVIN,  
OF LIMA, OHIO.

## METHOD OF AND APPARATUS FOR MAKING ELECTRIC STEEL.

Application filed April 28, 1920. Serial No. 377,197.

To all whom it may concern:

Be it known that I, JAMES W. GALVIN, a citizen of the United States, residing at Springfield, in the county of Clark and 5 State of Ohio, have invented certain new and useful Improvements in Methods of and Apparatus for Making Electric Steel, of which the following is a specification.

This invention relates to an improved 10 method of and apparatus for making electric steel.

One of the principal objects of my invention is the provision of an improved 15 method of and apparatus for producing steel in electric furnaces by virtue of which I am enabled to not only produce a given quantity of steel in less time and with much less power than is ordinarily required, but also to produce a product which is superior.

20 Another of the principal objects of my invention is to eliminate certain of the difficulties and disadvantages incident to the operation of standard electric melting furnaces.

25 My invention also contemplates the increase of the rated output of a standard furnace, about two to four times.

The foregoing, together with such other 30 objects as may hereinafter appear, or are incident to my invention, will be best understood from a brief description of standard practice, when taken in connection with the drawing, forming a part of this specification, and of which—

35 Figure 1 is a cross section through a standard tilting electric furnace, such as a Moore arc furnace, of three tons rated capacity; Figure 2 is a cross section through the same furnace as modified in accordance 40 with my invention; Figure 3 is a section illustrating the furnace of Figure 2, tilted to increase its capacity; and Figure 4 is a cross section illustrating how the capacity of a standard furnace may be still further 45 increased.

The structure shown in Figure 1, although specifically showing the Moore arc furnace, may be taken as a typical illustration of the standard practice in the art. 50 The bottom of the furnace is protected by a lining 7 of refractory material such as silica, such lining being built up to considerable depth so that the hearth 8 is relatively shallow and may be characterized 55 as being dish shaped. The side walls are

provided with openings for tapping the metal, such openings being closed by the doors 9. The electrodes are represented at 10 and it will be understood that they are operated automatically in the usual manner 60 so as to initially draw the arc and reestablish it when broken. Assuming that the furnace has a three ton rated capacity, the customary operation is as follows:

Three tons of scrap are charged into the 65 furnace. A small amount of pig iron or other carbonizer may be included in this charge or added thereto during the melting and in some cases in order to secure the proper chemical composition other elements 70 such as manganese ore, ferromanganese, ferro silicon, and the like may be added during the melting. When the current is first turned on, the electrodes are advanced until they engage the scrap and then they are 75 slightly retracted, drawing the arc. The scrap immediately adjacent to the electrodes is melted and the molten metal sinks to the bottom, and the electrodes, by virtue of 80 their automatic operation, follow down boring holes in the scrap. It will be readily understood by those skilled in the art that during this period, the arc will be frequently broken and the electrodes automatically shifted to reestablish the arc, as a result of 85 which the load fluctuations are very heavy. As the melting continues, the molten metal collects in a bath and the slag floating on the bath frequently breaks the arc and the electrodes are automatically lowered to re-establish it and the ends thereof immersed 90 in the slag. In fact, it is very common that the electrodes remain immersed in the slag after the arc has been reestablished. This is detrimental, for the reason that the 95 slag, by virtue of its higher resistance, immediately begins to boil violently and eats off the ends of the electrodes, as a result of which the metal absorbs the carbon, and also because the arc is too short. It will be 100 understood that the heavy load fluctuations above referred to take place during this period as well. After the charge is melted the entire charge is drawn off into the ladle as one batch, the furnace is recharged and 105 the operation repeated.

Another difficulty encountered in the operation of this type of furnace is that frequently it is found practically impossible to melt the scrap owing to the interstices be- 110

5 between pieces of scrap being so large as to prevent the formation of a suitable arc. It is furthermore commonly necessary, because of the shape of the hearth, to pull the 10 scrap into the bath of metal by using a hook or bar.

In addition to the foregoing, the power costs are high because the current and time requirements are relatively large. To overcome this and other disadvantages, I propose, briefly considered, to leave a portion of the molten metal in the furnace, when drawing off a batch during a run, and to add thereto a fresh charge, so that the latter 15 will absorb heat from the molten metal remaining in the furnace and the contents of the furnace will constitute a mass of great conductivity. In other words, enough molten metal is left to give the mass of 20 pieces of the succeeding charge conductivity to sustain the flow of current or arc between such charge and the superadjacent electrode means. This materially cuts down the power and the time required and secures other advantages which will appear. Such a process could not be carried out successfully in the standard furnace; but I have found that the furnace may be modified so as to carry out this process.

30 I have discovered that the lining 7 used in standard practice is more than twice as thick as is necessary for safety and proper radiation. This allows me, even while retaining the standard construction and con-

35 figuration in other respects, to construct the lining as shown in Figure 2, so as to produce a "cup-shaped" hearth 8, of deep-cupped or deep-rounded bowl profile, and with outward flare toward the furnace sides

40 sufficiently pronounced to cause unmolten material to gravitate even into the relatively narrow initial central pool or bath of molten metal on the hearth, and form therewith a mass of greater conductivity for sustaining the arc.

45 The capacity of the furnace is thus greatly increased; and it may be still further increased, if desired, by carrying the sidewalls of the lining to a higher level. By building the sidewalls upon one side

50 higher than the other, as shown, for example, in Figures 2, 3 and 4, at the right hand, the capacity of the furnace may be still further increased as will hereinafter appear.

55 When the sides of the lining are thus built up higher on one side than on the other, I prefer to correspondingly brick up the respective sides of the furnace wall proper, as shown in Figure 2, providing a

60 tap hole 9' in the lining and in the brick work of the high side below the level of the slag line, which hole is plugged with refractory sand 11, or the like. I also prefer to

construct the top of the side wall lining with no appreciable ledge.

65 I operate the furnace as thus modified as

to four times its original rated capacity of scrap, and then turn on the current and melt the entire charge. During the initial melting, when slag collects on the bath, interfering with the operation of the electrodes, I thin out the slag by adding a small amount of an oxidizer, such, for example, as iron ore, and slough off the thinned slag by tilting the furnace.

If the slag will not run out of the holes bored into the scrap 75 by the electrodes, I make an opening in the scrap by means of a bar or other suitable tool. As the melting continues and the bath of molten metal increases, the scrap will fall into the bath by virtue of the steep pitch or outward flare of the deep-cupped hearth and the sidewall linings; and little or no difficulty is encountered in maintaining the arc, because the contents of the furnace is a 85 more or less "solid" mass having excellent conductivity. Thus the heavy load fluctuations incident to the initiation of the melting are eliminated and care need be exercised only with respect to the removal of the slag, 90 at intervals, as may be required. To this end, as before, I occasionally add an oxidizer to thin out the slag to permit of its being readily sloughed off. In so far as I am aware, I am the first to do this in this 95 art, particularly in the acid electric process, which is the process I prefer.

When the initial charge has been completely melted I draw off only a portion of the melted charge as the first batch, preferably about one half, this being possible be-

cause of the increased capacity, and then I recharge into the remaining molten metal a quantity of scrap preferably sufficient to again fully charge the furnace, i. e., in the 100 case just supposed, about the same amount as left in the furnace. Thus the total content of the furnace is again two to four times the normal rated capacity of a stand-

ard furnace. This scrap sinks into the bath 105 and forms therewith a substantially "solid" or compact mass of relatively high or ample conductivity, so that the full efficiency of the current is obtained. If the scrap should

not sink freely because of slag remaining 110 on the bath of molten metal left in the fur-

nace as aforesaid, I thin out the slag as before, sloughing or drawing it off through the interstices amongst the pieces of the cold recharge just added, and thus 115 imparting some of its heat to the recharge.

In addition to the greater efficiency obtained by virtue of the fact that the mass has greater conductivity, it will be apparent 120 that less current and time will be required to melt the charge because the remaining molten metal will greatly assist in melting

the added charge. As before, from time to time, I remove the slag by first thinning it out; and when the charge is completely 125

- mented, I again draw off one half and refill or recharge the furnace. This cycle of periodic recharges, melting them and drawing off corresponding batches, and sloughing off slag during the process of fusion, etc., is repeated until the day's run is completed, when the last charge is completely drained off to permit of the repair of the lining, if required.
- 10 After the complete charge has been drawn off I charge the furnace while still hot with another extra large initial charge of some 16,000 to 20,000 pounds more or less of scrap, and leave it therein over night to absorb the heat of the furnace, so that on starting the next day's run less current and less time shall be required to melt the first charge,—the operation thereafter being as before stated.
- 20 To still further increase the capacity of the standard furnace, I prefer to tilt the furnace during operation, so that it will occupy a position such as shown in Figure 3, with its axis inclined to the vertical. This enables me to take advantage of the building up of one side of the furnace lining, a slight tilt serving to greatly increase the capacity of the furnace. The furnace is tilted to this position during the later stages 30 of the melting of a charge, say, for example, at the times when the scrap has become immersed in the bath.

It will be seen from the foregoing that I avoid the heavy load fluctuations ordinarily encountered because of the size shape and disposition of the scrap, at all times with the possible exception of the initial melting of the first charge of the day's run, and that by thinning out and sloughing off the slag during fusion of charges, etc., I obviate interference thereof with the passage of current or arc between the charge and the electrode means and the heavy load fluctuations due to that cause as well as the eating up of the electrodes normally encountered in standard practice. I am thus enabled not only to extend the life of the electrodes from two to three times beyond what may be ordinarily expected in standard practice, but also to produce a superior product. I am also able to increase the output as compared with that of an unmodified standard furnace operated in the usual manner; since with an initial charge of two to four times the original rated capacity of the furnace, a recharge even no more than half the initial charge, and a decreased duration of the fusion process due to the better electrical conditions, I can draw off molten batches at least as large as those of ordinary practice at shorter intervals.

Furthermore, by having the tap hole located at or below the slag line, when a charge is tapped the slag does not enter the ladle first as is usually the case in standard

practice and thus no impurities are absorbed from the slag as would otherwise occur. This is also advantageous when ladle additions are to be made.

I have further found in the operation of 70 standard furnaces, of the character described, that the brick work burns off as shown, for example, in Figure 4, and this, together with the fact that I have discovered that a much thinner lining may be employed, enables me to still further increase the capacity of the furnace.

In constructing new furnaces to operate in accordance with my invention, I construct the same with a deep hearth as set 80 forth and with the other requirements if desired.

I claim:

1. A method of electric steel production in molten batches through periodic melting 85 of corresponding charges by current passing between such charges and superjacent electrode means; which method comprises initially charging into the furnace and melting an extra large charge, and thereafter 90 smaller ones; leaving in the furnace, after each batch drawn off during a run, enough molten metal to give the mass of the succeeding charge conductivity to sustain the flow of current between the same and the 95 electrode means; and at the end of a run drawing off all the metal in the furnace and recharging it while still hot with an extra large initial charge for the next run, to absorb heat during the interval before such 100 next run.

2. A method of electric steel production through melting by current passing between the charge and superjacent electrode means; which method comprises thinning 105 and sloughing off slag during the process of fusion to obviate interference of such slag with passage of current between charge and electrode means.

3. A method of electric arc production 110 of molten steel according to the acid process; which method comprises sloughing off slag during the process of fusion to obviate interference of such slag with the arc.

4. A method of electric steel production 115 in molten batches through periodic melting of corresponding charges by current passing between such charges and superjacent electrode means; which method comprises leaving in the furnace, when drawing off a 120 batch enough molten metal to give the mass of the succeeding charge conductivity to sustain the flow of current between the same and the electrode means; and sloughing or drawing off through the interstices of such 125 succeeding charge slag remaining on the molten metal left in the furnace as aforesaid.

5. A method of electric steel production 130 in molten batches through periodic melting

of corresponding charges by current passing between such charges and superjacent electrode means; which method comprises leaving in the furnace, when drawing off a batch, enough molten metal to give the mass of the succeeding charge conductivity to sustain the flow of current between the same and the electrode means; and during fusion of charges sloughing off resulting slag to obviate interference thereof with the flow of current between charge and electrode means.

6. A method of electric arc production of steel in molten batches, according to the acid process, through periodic melting of corresponding charges; which method comprises initially charging into the furnace and melting an extra large charge, and thereafter smaller ones; leaving in the furnace, after each batch drawn off during a run, enough molten metal to give the mass of the succeeding charge conductivity to sustain the arc; sloughing off slag during fusion of charges to obviate interference thereof with the arc, and when slag remaining on the molten metal left in the furnace as aforesaid interferes with union of the recharge with such metal, sloughing or drawing off such slag through the interstices of the recharge; and at the end of a run drawing off all the metal in the furnace, and thereafter recharging it with an extra large initial charge for the succeeding run.

7. A method of electric arc production of

steel in molten batches, according to the acid process, through periodic melting of corresponding charges; which method comprises initially charging into the furnace and melting an extra large charge, and thereafter smaller ones; leaving in the furnace, after each batch drawn off during a run, enough molten metal to give the mass of the succeeding charge conductivity to sustain the arc; sloughing off slag during fusion of charges to obviate interference thereof with the arc, and when slag remaining on the molten metal left in the furnace as aforesaid interferes with union of the recharge with such metal, sloughing or drawing off such slag through the interstices of the recharge; and at the end of a run drawing off all the metal in the furnace, and thereafter recharging it with an extra large initial charge for the succeeding run.

In testimony whereof, I have hereunto signed my name.

JAMES W. GALVIN